

June 17, 1941.

A. S. BELL ET AL

2,245,641

COMPOSITE YARN AND FABRIC MADE OF OR CONTAINING SUCH YARN

Filed Oct. 3, 1939



FIG. 2



FIG. 3



FIG. 4



FIG. 5



FIG. 6



FIG. 7



A. S. BELL  
W. C. ANGUS  
INVENTORS

*J. Bell & C. Angus*  
ATTORNEYS

## UNITED STATES PATENT OFFICE

2,245,641

COMPOSITE YARN AND FABRIC MADE OF OR  
CONTAINING SUCH YARN

Angus Smith Bell and William Campbell Angus,  
Spondon, near Derby, England, assignors to  
Celanese Corporation of America, a corporation  
of Delaware

Application October 3, 1939, Serial No. 297,671  
In Great Britain November 9, 1938

13 Claims. (Cl. 57—144)

This invention relates to composite yarns, and fabrics of or containing such yarns.

Composite yarn according to the invention comprises a predominating component consisting of one or more voluminous crimped yarns of continuous filament origin doubled, by a substantial amount of doubling twist, with a base thread, the length of said predominating component being substantially greater than the length of said base thread, and a binding thread doubled about the assembly of the predominant component and the base thread. The voluminosity of the predominating component may be imparted thereto by false twisting a continuous filament yarn to a high or comparatively high degree in the presence of a setting agent (see, for example, U. S. Patents Nos. 2,089,198, 2,089,199 and 2,111,211 for methods of imparting crimps or crinkle to cellulose acetate or other cellulose derivative yarns by false twisting in the presence of steam) or by boiling flat filament cellulose derivative yarns.

The voluminous component, which may consist of one or more yarns in accordance with the bulk desired, is fed intermittently to a base thread and doubled therewith with a substantial amount of twist and a binding thread is doubled about the assembly, preferably with a moderate degree of twist in the reverse direction, so that the final composite thread exhibits large flakes of the voluminous yarn held firmly to the base thread by the binding thread. Preferably, the voluminous yarn amounts to about 70 or 80% or so by weight of the total weight of the composite yarn, due regard being had, however, to the provision of sufficient strength by way of the base and binding threads for the use to which the composite yarn is to be put. Preferably, the binding thread has a fairly high twist, and for this purpose a crepe thread may be used. The base thread may be of any suitable characteristics, for example a relatively low twist continuous filament thread may be used, e. g. a thread of cellulose acetate, but advantageously a stretched or a stretched and saponified cellulose acetate thread may be employed as the base, thus permitting adequate strength being obtained without undue weight in the base thread.

A further feature of the invention comprises fabrics made of or containing the composite yarns as above described. These fabrics employ a special type of weave, the principle of which is to give the composite yarns a series of long floats, together with a compact interlacing between the floats. The composite yarns may be

in the warp or weft or both, and may comprise the totality of the warp and/or weft or may be used in conjunction with other types of yarn.

By way of example, the construction of the type of yarn according to the invention, and some forms of fabric construction for utilising the yarn will now be described in greater detail with reference to the drawing accompanying the provisional specification, in which

10 Fig. 1 shows diagrammatically the construction of the yarn;

Figs. 2-5 show weaving diagrams suitable for fabrics containing the composite yarn in both warp and weft; and

15 Figs. 6 and 7 show weaving diagrams suitable for use with the composite yarn in the weft only.

Referring to Fig. 1, to a base thread 1 of low twist cellulose acetate filaments of say 100 to 150 denier, two 170-denier threads 2 of voluminous cellulose acetate are fed intermittently and twisted with the base thread to 40 turns per inch Z-twist. The rate of feed of the threads 2 is such that some 3-3½ inches of each of these threads are doubled with each one inch length of the thread 1. The result of the doubling is to produce flakes 3 of the voluminous yarn along the base thread 1. To secure the flakes in position a binding thread 4 of 100-150 denier viscose crepe (with 30 or so turns per inch S-twist) is doubled round the assembly with about 10 or 12 turns per inch S-twist.

Figs. 2-5 of the accompanying drawing show four forms of weave suitable for fabrics in which the composite yarns are used in both warp and weft. It will be seen in each case that both the warp yarns and the weft yarns float at intervals, but between the floats are securely interlaced with each other.

20 Figs. 6 and 7 show weaves suitable for the use of the composite yarn in the weft only, the warp being composed of plain yarns of fine deniers. Here again, the weft yarns will be seen to float with secure interlacings between each float. A special feature of the fabrics woven according to 25 Figs. 6 and 7 is that the main effect of the composite yarn is thrown on to the face of the fabric.

Fabrics woven as just described show an astrakhan or similar fur-like appearance, or in some cases have a cloqué effect because of the protuberance of the long flakes of the voluminous material in the composite yarns. When a crêpe thread is used as the binder, the shrinkage of this thread further accentuates the flaky characteristics of the composite yarn, and also imparts a 30 compactness to the finished fabrics.

Having described our invention, what we desire to secure by Letters Patent is:

1. A composite yarn, comprising a predominating component consisting of one or more low twist voluminous crimped yarns of continuous filament origin doubled, by a substantial amount of doubling twist, with a base thread, the length of said predominating component being substantially greater than the length of said base thread, and a binding thread doubled with a smaller amount of doubling twist about the assembly of the predominant component and the base thread. 5
2. A composite yarn, of which at least 70% by weight is constituted by a predominating component consisting of at least one low twist voluminous crimped yarn of continuous filament origin, said composite yarn comprising also a base thread substantially shorter in length than said crimped yarn and doubled by a substantial amount of doubling twist with said crimped yarn, and a binding thread doubled with a smaller amount of doubling twist about the assembly of said crimped yarn and said base thread. 10
3. A composite yarn, of which at least 70% by weight is constituted by a predominating component consisting of at least one low twist voluminous crimped yarn of continuous filament origin, said composite yarn comprising also a base thread substantially shorter in length than said crimped yarn and doubled by a substantial amount of doubling twist with said crimped yarn, and a binding thread having a high degree of twist and doubled with a smaller amount of doubling twist about the assembly of said crimped yarn and said base thread. 15
4. A composite yarn, of which at least 70% by weight is constituted by a predominating component consisting of at least one low twist voluminous crimped yarn of continuous filament origin, said composite yarn comprising also a base thread substantially shorter in length than said crimped yarn and doubled by a substantial amount of doubling twist with said crimped yarn, and a crepe twisted binding thread doubled with a smaller amount of doubling twist about the assembly of said crimped yarn and said base thread. 20
5. A composite yarn, of which at least 70% by weight is constituted by a predominating component consisting of at least one low twist voluminous crimped yarn of continuous filament origin, said composite yarn comprising also a low-twist continuous filament base thread substantially shorter in length than said crimped yarn and doubled by a substantial amount of doubling twist with said crimped yarn, and a binding thread doubled with a smaller amount of doubling twist about the assembly of said crimped yarn and said base thread. 25
6. A composite yarn, of which at least 70% by weight is constituted by a predominating component consisting of at least one low twist voluminous crimped yarn of continuous filament origin, said composite yarn comprising also a stretched continuous filament low-twist thread of an organic derivative of cellulose substantially shorter than said crimped yarn, constituting a base thread doubled by a substantial amount of doubling twist with said crimped yarn, and a binding thread doubled with a smaller amount of doubling twist about the assembly of said crimped yarn and said base thread. 30
7. A composite yarn, of which at least 70% by weight is constituted by a predominating component consisting of at least one low twist voluminous crimped yarn of continuous filament origin, 35

said composite yarn comprising also a stretched and saponified continuous filament low-twist thread of cellulose acetate substantially shorter than said crimped yarn, constituting a base thread doubled by a substantial amount of doubling twist with said crimped yarn, and a binding thread doubled with a smaller amount of doubling twist about the assembly of said crimped yarn and said base thread.

8. A composite yarn, of which at least 70% by weight is constituted by a predominating component consisting of a plurality of low twist voluminous crimped yarns of continuous filament origin, said composite yarn comprising also a base thread substantially shorter in length than said crimped yarns and doubled by a substantial amount of doubling twist with said crimped yarns, and a binding thread doubled with a smaller amount of doubling twist about the assembly of said crimped yarns and said base thread. 40

9. A composite yarn, of which at least 70% by weight is constituted by a predominating component consisting of a plurality of low twist voluminous crimped yarns of continuous filament origin, said composite yarn comprising also a stretched continuous filament low-twist thread of an organic derivative of cellulose substantially shorter than said crimped yarns, constituting a base thread doubled by a substantial amount of doubling twist with said crimped yarns, and a binding thread doubled with a smaller amount of doubling twist about the assembly of said crimped yarns and said base thread. 45

10. A composite yarn, of which at least 70% by weight is constituted by a predominating component consisting of a plurality of low twist voluminous crimped yarns of continuous filament origin, said composite yarn comprising also a stretched and saponified continuous filament low-twist thread of cellulose acetate substantially shorter than said crimped yarns constituting a base thread doubled by a substantial amount of doubling twist with said crimped yarns, and a binding thread doubled with a smaller amount of doubling twist about the assembly of said crimped yarns and said base thread. 50

11. A woven fabric containing in its woven structure composite yarns each comprising a predominating component consisting of one or more low twist voluminous crimped yarns of continuous filament origin doubled by a substantial amount of doubling twist, with a base thread, the length of said predominating component being substantially greater than the length of said base thread, and a binding thread doubled with a smaller amount of doubling twist about the assembly of the predominant component and the base thread, said composite yarns being given in the fabric a series of long floats alternating with periods of compact interlacing in the fabric. 55

12. A woven fabric containing as part of its woven structure composite yarns of each of which at least 70% by weight is constituted by a predominating component consisting of a plurality of low twist voluminous crimped yarns of continuous filament origin, said composite yarns comprising also a stretched continuous filament low-twist thread of an organic derivative of cellulose substantially shorter than said crimped yarns, constituting a base thread doubled by a substantial amount of doubling twist with said crimped yarns, and a binding thread doubled with a smaller amount of doubling twist about the assembly of said crimped yarns and said base thread, said composite yarns being given in the fabric a series 60

of long floats alternating with periods of compact interlacing in the fabric.

13. A woven fabric containing as part of its woven structure composite yarns of each of which at least 70% by weight is constituted by a predominating component consisting of a plurality of low twist voluminous crimped yarns of continuous filament origin, said composite yarns comprising also a stretched and saponified continuous filament low-twist thread of cellulose acetate substantially shorter than said crimped yarns con-

stituting a base thread coupled by a substantial amount of doubling twist with said crimped yarns, and a binding thread doubled with a smaller amount of doubling twist about the assembly of said crimped yarns and said base thread said composite yarns being given in the fabric a series of long floats alternating with periods of compact interlacing in the fabric.

10

ANGUS SMITH BELL.  
WILLIAM CAMPBELL ANGUS.